

## UNITED STATES PATENT OFFICE

2,278,747

## CHEMICAL COMPOSITION

Fenton H. Swezey, Morris Earl Bishop, and Robert M. Hoffman, Waynesboro, Va., assignors to E. I. du Pont de Nemours & Company, Wilmington, Del., a corporation of Delaware

No Drawing. Application May 23, 1940,  
Serial No. 336,890

1 Claim. (CL 252—8.75)

This invention relates to an improved dressing composition for lubricating, softening and/or flexibilizing filaments, yarns, threads, or the like comprised of organic acid esters of cellulose, together with filaments, yarns, threads, and the like to which the composition has been applied; and more particularly to an improved stable, antistatic, and non-corrosive composition comprising palm kernel oil for lubricating, softening and/or flexibilizing filaments, yarns, threads, and the like comprised of cellulose acetate, together with filaments, yarns, threads, and the like of cellulose acetate to which the composition has been applied.

It is a desirable and necessary practice to treat filaments, yarns, thread, and the like produced from organic esters of cellulose with a dressing composition prior to initial collection in package form of such filament, yarn or thread. Formulation of a satisfactory composition is fraught with difficulties for in addition to lubricating, softening and/or flexibilizing the filaments, a suitable dressing composition must fulfill additional functions. It is well known, for example, that filaments of organic acid esters of cellulose become readily charged with static electricity which is troublesome in subsequent operations, and it is necessary therefore to have in the dressing composition an ingredient to neutralize this charge, or minimize its effect. Further, it is known that vegetable oils, otherwise satisfactory as lubricating and softening agents tend to oxidize upon ageing and these oxidized compounds deleteriously affect the filament, yarn or thread. Hence, the dressing composition must contain a constituent to prevent oxidation of the softening agent. And to complicate matters further, fresh spun filaments of organic acid esters of cellulose produced by the evaporative spinning method, for example cellulose acetate produced by the spinning of acetone-soluble cellulose acetate dissolved in acetone, have the peculiar property of occluding ingredients from finishing compositions when applied thereto immediately after leaving the spinning cell and prior to initial collection in package form. This occlusion of finish composition affects the filament variously in that fabrics produced therefrom dye non-uniformly; also the luster of the filament is frequently affected, and unfortunately non-uniformly.

It has therefore been extremely difficult to compound a suitable dressing composition which will have the requisite softening and lubricating action on the filament, yarn or thread, which

will minimize static effect, prevent oxidation of the softening agent, and still have a finish that will not be occluded but will uniformly affect the filament, and can be readily and uniformly removed therefrom after fabrication of the filament, yarn or thread into a fabric.

This invention has as an object new dressing compositions particularly suited for treating filaments, yarns and threads composed of organic acid esters of cellulose. A further object is the production of dressing compositions free of constituents which are occluded by fresh-spun filaments of organic acid esters of cellulose. A still further object is the production of dressing compositions which do not oxidize with age, which neutralize or minimize the effect of the static charge, and which at the same time uniformly lubricate and soften filaments of organic acid esters of cellulose. A still further object is the formulation of a dressing composition which will impart a uniform finish to cellulose acetate filaments, yarns and threads. A still further object resides in the filaments, yarns and threads of organic acid esters of cellulose to which our novel dressing compositions have been applied. These and other objects will more clearly appear hereinafter.

These objects are accomplished by the following invention. It has been found that palm kernel oil is outstanding as a softening and lubricating agent for filaments, yarns and threads of organic acid esters of cellulose and particularly for cellulose acetate yarn. It has a low iodine number, or in other words, it is relatively free from unsaturated compounds and, therefore, is less apt to develop odor and rancidity upon storage as compared to other non-drying vegetable oils such as olive oil. Additionally, palm kernel oil is not occluded or dissolved in the filament, yarn or thread, and compositions containing a large proportion of palm kernel oil can be more readily removed from fabricated yarn products and the like than has been possible with compositions used heretofore.

It has further been found that palm oil combined with known antistatic materials, corrosion inhibitors, antioxidants and diluents in the following proportions by weight:

|                        | Parts |
|------------------------|-------|
| Palm kernel oil        | 100   |
| An antistatic material | 5-15  |
| Corrosion inhibitor    | 0.1-1 |
| An antioxidant         | 0.5-5 |
| Diluent                | 0-150 |

constitutes an exceptionally good dressing composition for softening, lubricating, and/or flexibilizing filaments, yarns, threads or the like, produced from organic acid esters of cellulose such as cellulose acetate.

It is, of course, desirable to use a high grade palm kernel oil of light color and uniform physical characteristics from lot to lot. As the antistatic material, compounds falling under the term "N-dialkylcyclohexylamine 'lorol' sulfate" such as dimethylcyclohexylamine "lorol" sulfate and diethylcyclohexylamine "lorol" sulfate, have proven very satisfactory. The term "lorol" is intended to cover the residue of the commercially available mixed primary alcohols containing 10 to 18 carbon atoms. In addition, the products described in U. S. Patent No. 2,139,276 to Lenher et al., such as diethylcyclohexylamine lauryl sulfate, dimethylcyclohexylamine lauryl sulfate, diethylcyclohexylamine stearyl sulfate, diethylcyclohexylamine cetyl sulfate, etc., have also proven very satisfactory. Other suitable materials for this purpose are a 50-50 mixture of sodium "ocenol" (commercially available mixed unsaturated alcohols containing 16 and 18 carbon atoms) sulfate and sodium cetyl sulfate, trimethylstearyl ammonium bromide, "Stenol," which is a mixture of the higher alcohols comprising chiefly alcohols containing 16 and 18 carbon atoms with a little alcohol of 14 carbon atoms, and the reaction product of dialkanol stearamide and dimethyl sulfate such as the reaction product of diethanol stearamide and dimethyl sulfate. As the corrosion inhibitor, "dilrol" phosphate, diethylcyclohexylamine, lecithin, and triethanolamine have been found quite satisfactory. Any well known antioxidants such as hydroquinone, alpha naphthol, beta naphthol, Eugenol, diphenylamine, lecithin, and pyrogallol may be used. Mixtures of two or more of the above antistatic agents, mixtures of two or more antioxidants, and mixtures of two or more corrosion inhibitors may of course be employed. The diluent is preferably a refined mineral oil and should preferably be of low viscosity. Other diluents such as kerosene, diethylene glycol monolaurate, and butyl palmitate also be used.

As specific examples which have been found exceptionally suitable and particularly for dressing cellulose acetate multi-filament yarn, the following are given; parts are by weight:

#### Example I

|                                                             | Parts |
|-------------------------------------------------------------|-------|
| Palm kernel oil                                             | 100   |
| Diethyl cyclohexylamine "lorol" sulfate as antistatic agent | 5.5   |
| "Dilrol" phosphate as the corrosion inhibitor               | 0.2   |
| Eugenol as the antioxidant                                  | 0.83  |
| Kerosene as the diluent                                     | 5.5   |

#### Example II

|                                                                | Parts |
|----------------------------------------------------------------|-------|
| Palm kernel oil                                                | 100   |
| Diethylcyclohexylamine "lorol" sulfate as the antistatic agent | 7.8   |
| Diethylcyclohexylamine as the corrosion inhibitor              | 0.8   |
| "Dilrol" phosphate as the corrosion inhibitor                  | 0.17  |
| Eugenol as the antioxidant                                     | 0.8   |
| Lecithin also as the antioxidant                               | 3.3   |
| Refined mineral oil as the diluent                             | 52    |
|                                                                | 75    |

#### Example III

|                                                                | Parts |
|----------------------------------------------------------------|-------|
| Palm kernel oil                                                | 100   |
| Diethylcyclohexylamine "lorol" sulfate as the antistatic agent | 5     |
| "Dilrol" phosphate as the corrosion inhibitor                  | 0.2   |
| Eugenol as the antioxidant                                     | 1     |

#### Example IV

|                                                                | Parts |
|----------------------------------------------------------------|-------|
| Palm kernel oil                                                | 100   |
| Diethylcyclohexylamine stearyl sulfate as the antistatic agent | 5     |
| Lecithin as the corrosion inhibitor                            | 1     |
| Hydroquinone as the antioxidant                                | 1     |

#### Example V

|                                                              | Parts |
|--------------------------------------------------------------|-------|
| Palm kernel oil                                              | 100   |
| Diethylcyclohexylamine cetyl sulfate as the antistatic agent | 10    |
| Triethanolamine as the corrosion inhibitor                   | 1     |
| Alpha naphthol as the antioxidant                            | 2     |
| Refined mineral oil as the diluent                           | 100   |

#### Example VI

|                                                                                           | Parts |
|-------------------------------------------------------------------------------------------|-------|
| Palm kernel oil                                                                           | 100   |
| Equal mixture of sodium "ocenol" sulfate and sodium cetyl sulfate as the antistatic agent | 5     |
| "Dilrol" phosphate as the corrosion inhibitor                                             | 0.1   |
| Beta naphthol as the antioxidant                                                          | 0.5   |

#### Example VII

|                                                            | Parts |
|------------------------------------------------------------|-------|
| Palm kernel oil                                            | 100   |
| Trimethyl stearyl ammonium bromide as the antistatic agent | 5     |
| "Dilrol" phosphate as the corrosion inhibitor              | 0.1   |
| Diphenylamine as the antioxidant                           | 1     |

#### Example VIII

|                                                                                                                                                                                                                                                          | Parts |
|----------------------------------------------------------------------------------------------------------------------------------------------------------------------------------------------------------------------------------------------------------|-------|
| Palm kernel oil                                                                                                                                                                                                                                          | 100   |
| A 25% solution of the reaction product of stearic acid and diethanolamine prepared as described in the first part of Example 7 of U. S. Patent 2,096,749 and then treated with dimethyl sulfate as described in the same patent, as the antistatic agent | 5     |
| "Dilrol" phosphate as the corrosion inhibitor                                                                                                                                                                                                            | 0.1   |
| Eugenol as the antioxidant                                                                                                                                                                                                                               | 1     |

#### Example IX

|                                                                                                                                                                                                                                                          | Parts |
|----------------------------------------------------------------------------------------------------------------------------------------------------------------------------------------------------------------------------------------------------------|-------|
| Palm kernel oil                                                                                                                                                                                                                                          | 100   |
| A 25% solution of the reaction product of stearic acid and diethanolamine prepared as described in the first part of Example 7 of U. S. Patent 2,096,749 and then treated with dimethyl sulfate as described in the same patent, as the antistatic agent | 5     |
| "Dilrol" phosphate as the corrosion inhibitor                                                                                                                                                                                                            | 0.1   |
| Lecithin as the antioxidant                                                                                                                                                                                                                              | 1     |
| Eugenol as the antioxidant                                                                                                                                                                                                                               | 2     |

## Example X

Palm kernel oil.....  
 A 25% solution of the reaction product of stearic acid and diethanolamine prepared as described in the first part of Example 7 of U. S. Patent 2,096,749 and then treated with dimethyl sulfate as described in the same patent, as the antistatic agent.....  
 "Dilrol" phosphate [as the corrosion inhibitor].....  
 Diethylcyclohexylamine [as the antioxidant].....  
 Eugenol as the antioxidant.....  
 Refined mineral oil as the diluent.....

## Example XI

Palm kernel oil.....  
 A 25% solution of the reaction product of stearic acid and diethanolamine prepared as described in the first part of Example 7 of U. S. Patent 2,096,749 and then treated with dimethyl sulfate as described in the same patent, as the antistatic agent.....  
 Eugenol as the antioxidant.....  
 "Dilrol" phosphate as the corrosion inhibitor.....  
 Refined mineral oil as the diluent.....

Any convenient procedure for mixing the ingredients set forth in the foregoing compositions can be used. It is generally desirable to heat the palm kernel oil to about 40°-50° C. to render it completely liquid. (Its melting point is in the neighborhood of 30° C.) While agitating and maintaining a temperature between about 40°-50° C., the antistatic material is added, and after stirring this mixture for a few minutes the other ingredients, preferably in the following order, are added: the diluent, corrosion inhibitor, and the antioxidant. Throughout this mixing the temperature is maintained above about 40° C. and the mixture agitated. When mineral oil is used as the diluent, it is frequently desirable to dissolve the antioxidant, for example lecithin, therein and then incorporate this mixture in the palm kernel oil-antistatic agent mixture.

It is, of course, understood that while this invention has been described specifically as a dressing composition for cellulose acetate yarn, it is suitable for use with other organic acid esters of cellulose, such as on filaments, yarn, threads, and the like produced from cellulose propionate, cellulose butyrate, cellulose aceto-propionate, cellulose aceto-butyrate, etc. It may be applied not only to continuous filament yarn which will be sold and used as such, but also to ropes of continuous filaments which will subsequently be cut or otherwise formed into staple.

The filament, yarn or thread may be treated with this finish in any suitable manner, such as by means of wiper rolls in contact with the finish

Parts 100 and also in contact with the yarn or the like, by means of wicks or by other means known to those skilled in the art. The yarn will preferably be treated so that it contains from 0.5% to 10% by weight of the composition of this invention and more generally from 1.0% to 3.0% of this composition.

Parts 10 10 The physical properties of palm kernel oil with regard to melting point, viscosity, or some other characteristics, are such that the physical quality of the yarn and the like processed with the dressing composition described herein is better than that of yarn processed with finishes made substantially from mineral oil or other vegetable oils such as olive oil. This improved physical quality of the yarn may come about from a better cohesion of the filaments with increased protection from abrasion, and results in greater freedom from loops, broken filaments, fluff, or other common yarn defects.

Parts 100 15 20 The use of palm kernel oil avoids the deleterious oxidation effects associated with the high percentage of unsaturated chemical bonds present in the usual vegetable oils heretofore used in textile processing. Oxidation results in uneven dyeing and reduced tensile strength for the yarns involved. Oxidation can occur on storage, and is accelerated by exposure to radiation such as heat and light, or oxidizing agents such as ozone. Palm kernel oil finishes possess a very desirable resistance to these influences.

Parts 7 25 30 35 Cellulose acetate yarn which has been impregnated by the compositions above described can be readily knit in the usual manner without difficulty and the knit goods so produced can be easily freed from the dressing composition without deleteriously affecting the yarn. More particularly, the yarn so finished is exceptionally useful as filling yarn in woven goods and can be readily twisted and wound in any suitable form.

Parts 1.5 25 30 35 40 45 It is to be understood that the above description is for purposes of illustration, and that the invention is not limited thereby but includes rather all modifications and equivalents falling under the terms and spirit thereof as set forth in the following claim.

We claim:

50 55 A dressing composition to be applied to filaments, yarns and threads of cellulose acetate which comprises about 100 parts by weight of palm kernel oil, about 7.8 parts of diethylcyclohexylamine "loral" sulfate, about 0.8 part of diethylcyclohexylamine, about 0.17 part of "dilrol" phosphate, about 0.8 parts of Eugenol, about 3.3 parts of lecithin, and about 52 parts of refined mineral oil.

FENTON H. SWEZEEY.  
 MORRIS EARL BISHOP.  
 ROBERT M. HOFFMAN.

## CERTIFICATE OF CORRECTION.

Patent No. 2,278,747.

April 7, 1942.

FENTON H. SWEZYEY, ET AL.

It is hereby certified that error appears in the printed specification of the above numbered patent requiring correction as follows: Page 2, first column, line 48, before "also" insert --may--; and second column, line 74, for "Lecithin" read --Eugenol--; line 75, for "Eugenol" read --Lecithin--; page 3, first column, line 43, for "lechithin" read --lecithin--; and second column, line 45, for "raher" read --rather--; line 53, for "loral" read --lorol--; line 56, for "parts or" read --parts of--; and that the said Letters Patent should be read with this correction therein that the same may conform to the record of the case in the Patent Office.

Signed and sealed this 26th day of May, A. D. 1942.

(Seal)

Henry Van Arsdale,  
Acting Commissioner of Patents.

CERTIFICATE OF CORRECTION.

Patent No. 2,278,747.

April 7, 1942.

FENTON H. SWEZEY, ET AL.

It is hereby certified that error appears in the printed specification of the above numbered patent requiring correction as follows: Page 2, first column, line 48, before "also" insert --may--; and second column, line 74, for "Lecithin" read --Eugenol--; line 75, for "Eugenol" read --Lecithin--; page 3, first column, line 43, for "lechithin" read --lecithin--; and second column, line 45, for "raher" read --rather--; line 53, for "loral" read --lorol--; line 56, for "parts or" read --parts of--; and that the said Letters Patent should be read with this correction therein that the same may conform to the record of the case in the Patent Office.

Signed and sealed this 26th day of May, A. D. 1942.

(Seal)

Henry Van Arsdale,  
Acting Commissioner of Patents.